

Feb. 9, 1943.

J. DORNAUF

2,310,766

## CASTING METAL

Filed Oct. 17, 1939

2 Sheets-Sheet 1

Fig. 1



Inventor:

**JOSEF DORNAUF,**

*By*

Barney D. Larson  
ATTORNEYS

Feb. 9, 1943.

J. DORNAUF

2,310,766

CASTING METAL

Filed Oct. 17, 1939

2 Sheets-Sheet 2



Fig. 2.

Fig. 3.



Load Periods in Millions

Fig. 4.

INVENTOR  
JOSEF DORNAUF,

By *Barley & Larson*  
ATTORNEYS

## UNITED STATES PATENT OFFICE

2,310,766

## CASTING METALS

Josef Dormauf, Frankfort-on-the-Main, Germany; vested in the Alien Property Custodian

Application October 17, 1939, Serial No. 299,881  
In Germany December 7, 1938

6 Claims. (Cl. 22—209)

This invention is directed to the casting of metals, and especially to the casting of metals under pressure to reduce the porosity of the cast solidified metal.

Prior to this invention, many attempts have been made to eliminate or reduce the porosity of metal castings, particularly light metal castings including aluminum and aluminum alloys. Such methods as pouring molten metal into a mold, and then subjecting it to great mechanical or other pressure, have been without success. In particular, a practical method of casting alloys of aluminum with silicon has not been known, as known methods produced castings which had their advantages of decreased porosity offset by the creation of enlarged internal cavities.

The production of dense castings free from pores is especially desirable for delicate castings which must be machined and used, for example, as aircraft motor housings. Particular difficulty has existed in the casting of Al-Si alloys modified with sodium, wherein the porosity of the casting is not altogether caused by the gases developed in the melt, as in the castings produced from ordinary metals and alloys thereof. Great waste has heretofore existed because many castings had to be discarded as being too porous, and thus too weak. As shapes machined from such castings are often used in places where they are subjected to vibration, it is very important to obtain a dense casting of great durability and resistance to fatigue.

It is an object of this invention to produce a dense casting.

A further object of the invention is to produce a very dense casting from light metals, especially such metals as aluminum or aluminum alloys.

A further object of the invention is to develop a practical method of casting alloys of aluminum and silicon, especially when modified with sodium, so that a very dense casting is obtained.

A further object of this invention is to produce a novel process of casting light metals under pressure wherein both the casting crucible and the mold and the metals in the crucible and mold are placed under substantially the same increased pressure and castings are obtained which are substantially free of pores, can be readily machined, and have unexpectedly great strength.

Generally, these objects of the invention are obtained by placing both the crucible containing the melt and the mold under pressure, which can amount to as great as 20 atmospheres in excess of atmospheric pressure, and causing the molten metal to flow from the crucible into the mold while both are subjected to this pressure. This process differs from the prior art methods in

that both the metal in the melting pot and the mold are under the same pressure, whereas in known former methods, the metal in the mold alone had an increased pressure applied to it after the metal had been poured therein.

5 The process in this invention is described in greater detail in connection with the accompanying drawings, in which:

Fig. 1 is a cross-sectional view of an apparatus which may be employed in the use of the casting process of this invention.

10 Fig. 2 is a photomicrograph of a casting produced by this invention.

Fig. 3 is a photomicrograph of a casting of metal similar to that of Fig. 2, but cast by conventional methods.

15 Fig. 4 is a diagram of Wöhler curves comparing metals cast by an old method and by this invention.

20 In Fig. 1, a pressure chamber is shown which consists of a housing 1, having a removable top 2 secured to housing 1 by bolts 2a. Compressed air, or other gas, is admitted into the chamber through pipe and valve 3. Safety valve 4 and pressure gauge 5 are connected to the chamber at any convenient plate, as through cover 2. A mold 6, shown as an ordinary sand mold, is placed within the pressure chamber. Before top 2 is put in place, a crucible 7 containing molten metal 7a therein, is lowered into place on top of the mold and surrounded by a protective insulating shield 8, which may be of asbestos. It is preferable to have the crucible 7 preheated before the molten metal is poured therein and lowered into the chamber. Crucible 7 includes a removable plug 8 in the bottom thereof, which plug is connected by pin 8a to a handle 8b extending through cover 2. After the crucible 7 has been placed within the chamber and the handle 8b connected to plug 8, air, or other pressure producing medium, is admitted into the chamber through valve 3. A pressure ranging from 5 to 20 atmospheres in excess of atmospheric pressure is built up within the chamber before plug 8 is pulled and the metal allowed to flow into the mold. It is noted that the pressure is applied to the metal in both the crucible and the mold. After the metal has solidified in the mold, the pressure is released from the chamber and the mold removed therefrom.

45 Repeated tests have proved that this method of casting is applicable to alloys of varying composition, and is a practical method for foundry use. No difficulty is experienced in pouring the melt into the mold, and there is no chance of the melt partially solidifying in the mold before the pressure is applied. Thus a uniformly increased density throughout the whole casting is obtained.

50 For example, bars having a diameter of 40 mm.

were cast at a pressure of 8 atmospheres in excess of atmospheric pressure. Comparative tests, as set forth in the table below, were run. Bars were cast according to conventional methods and according to the present invention, both forms of bars being cast from the same batch of molten metal and under the same conditions except those relating to the pressure. Test pieces were machined from these cast bars, and the test pieces from the bars cast under pressure showed an improved dense surface. Table I gives the composition of the alloy, and Table II shows the breaking strength of the bars.

Table I

| Alloy No. | Designation                    | Zn       | Cu       | Mg       | Si       | Ni       | Mn       | Sb       | Fe       | Tl       |
|-----------|--------------------------------|----------|----------|----------|----------|----------|----------|----------|----------|----------|
| 1         | Al-Mg alloy                    | Per cent | Per cent | Per cent | Per cent | Per cent | Per cent | Per cent | Per cent | Per cent |
| 2         | Y-alloy with special additions | ---      | ---      | 7        | 1        | ---      | ---      | 0.3      | ---      | ---      |
| 3         | Y-alloy                        | 2.25     | 1.6      | 1.25     | 1.3      | 1.4      | ---      | 0.3      | 0.1      | ---      |
| 4         | German alloy                   | 4        | 1.5      | ---      | 2        | ---      | ---      | 0.3      | ---      | ---      |
| 5         | Alloy resistant to seawater    | 10       | 2        | 0.5      | ---      | ---      | ---      | 0.5      | ---      | ---      |
|           |                                |          |          |          |          |          |          |          |          |          |
|           |                                | 2.3      | 0.6      | ---      | 1.5      | 0.2      | 0.3      | ---      |          |          |

The remainder of each of alloys 1 through 5 was aluminum.

Table II

| Alloy No. | Casting pressure in atmospheres in excess of atmospheric pressure | Tensile strength $\sigma_B$ kg./mm. <sup>2</sup> |
|-----------|-------------------------------------------------------------------|--------------------------------------------------|
| 1         | 8                                                                 | 14.0                                             |
| 2         | 0                                                                 | 9.5                                              |
| 3         | 8                                                                 | 24.0                                             |
| 4         | 0                                                                 | 15.2                                             |
| 5         | 8                                                                 | 23.0                                             |
|           | 0                                                                 | 20.3                                             |
|           | 8                                                                 | 17.4                                             |
|           | 0                                                                 | 14.8                                             |
|           | 0                                                                 | 12.8                                             |
|           | 0                                                                 | 11.4                                             |

It is clear from the results set forth in the tables that remarkable increases in tensile strength were obtained in each instance where the bar was cast according to the new method. The increased density of the castings permitted machined shapes to be produced which had firm dense surfaces.

A particularly advantageous discovery of the invention lies in that increased density is obtained in casings of aluminum silicon alloys which are modified with sodium, it being noted that the sodium gives a porosity which is entirely different from the usual piping or porousness caused by imprisoned gases in the casting. This particular porosity occurs in the interior of the casting, while the outside surface is dense, and the porous interior is exposed when the casting is machined. Thus, aluminum silicon alloys modified with sodium, while very desirable for delicate castings, have been very expensive in view of the waste incurred in the machining of the castings, which necessitated the remelting of a great many castings. Even the addition of salts having a degasifying effect upon the melt failed to improve materially the denseness of the interior of the castings. Again, the most improved aluminum silicon alloys with further ad-

ditions of Mg, Mn, and the like, were too porous to be completely successful.

It was discovered that when such aluminum silicon alloys modified with sodium were cast according to this invention, a remarkably dense casting was obtained. For example, an alloy composed of

|           | Percent   |
|-----------|-----------|
| Si        | 12.5      |
| Mg        | 0.3       |
| Manganese | 0.5       |
| Al        | Remainder |

was melted at a temperature of 780° C. and was treated with 0.06% Na. Immediately after the addition of sodium, the melt was poured into a preheated crucible, and the crucible placed together with the mold in a pressure chamber. A pressure of 5 atmospheres in excess of atmospheric pressure was built up in the chamber before the plug was drawn from the crucible and the molten metal flowed into a sand mold. The casting was removed from the mold after it had solidified.

Fig. 2 is a photomicrograph of a section of the casting thus obtained. This casting is substantially free of pores, and is very dense.

In comparison with this casting of the aluminum silicon alloy treated with sodium, a similar casting was made of the same dimensions and composition, with the casting being done by conventional methods. Care was taken that the melting and the casting operation and also the time periods before and after the addition of sodium and the method of pouring the metal into the mold were exactly the same as the pressure casting test. In other words, the same test was run, except that both the crucible and mold were not put under an increased pressure. The result of this test is shown in Fig. 3, which is a photomicrograph of a section of the bar obtained. This photomicrograph shows many pores in the casting. By comparing Fig. 2 with Fig. 3, it is clear that the casting according to this invention, that is casting under a pressure of 5 atmospheres in excess of atmospheric pressure, produced a casting much denser than the casting shown in Fig. 3.

Aluminum alloys with from 0.5 to 15% silicon are beneficially treated by this method, it being noted that the best results are obtained with the eutectic alloys containing from 8% to 15% silicon.

The strength of the bars cast under pressure is increased as well as the density. Tests have shown that under otherwise equal conditions, the strength of bars cast under pressure is increased from 6.5 kg./mm.<sup>2</sup> to 9.5 kg./mm.<sup>2</sup> over bars cast according to conventional methods. The test bars were machined from sand castings having a thickness of 40 mm.

The results of fatigue tests are shown more clearly in Fig. 4. In this figure, the Wöhler curves are plotted from bars cast from a single melt. The alloy consisted of

|    | Per cent  |
|----|-----------|
| Si | 12.5      |
| Mg | 0.3       |
| Mn | 0.5       |
| Al | Remainder |

The melt was treated with sodium before the casting. Bars 40 mm. thick were cast in sand. Curve A represents the fatigue strength of the bars cast under a pressure of 5 atmospheres in excess of atmospheric pressure according to the novel process of this invention, and curve B rep-

sents the same test of fatigue strength for the parts cast at atmospheric pressure by old methods. Comparison of the curves shows that for all loads and for all periods of load application, the test pieces cast under pressure according to the present invention are superior.

It has therefore been shown that by the instant invention, delicate castings can be obtained, particularly from light metals, which can be used in places requiring lightness as well as durability, resistance to fatigue, and strength. As these castings can be machined without exposing porous surfaces, a great savings is obtained over castings produced by other known methods.

Therefore, it is evident that great advantages are obtained by placing both the crucible and the mold under the same pressure before pouring,asmuch as no additional skill is required in pouring the melt into the mold, and no time lag exists between the pouring and the application of pressure. The method is simple, and of practical use in a foundry.

Having now described a means by which the objects of this invention may be obtained, what I claim as new and desire to secure by Letters Patent is:

1. A process of casting metals under pressure from a crucible to a mold which comprises passing molten metal from the crucible to the mold while simultaneously subjecting the metal in the crucible and in the mold to a pressure of at least five atmospheres in excess of atmospheric pressure.

2. A process of casting light metal alloys to form castings substantially free from pores and of great fatigue strength comprising pouring molten metal into a mold while simultaneously subjecting both the metal being poured and the mold to substantially the same increase in atmos-

pheric pressure amounting to at least 5 atmospheres.

3. A process of casting metals which comprises placing a crucible containing molten metal, and a mold for receiving the molten metal, within a pressure chamber, creating a pressure of at least five atmospheres in excess of atmospheric pressure within said chamber, and pouring the metal from the crucible into the mold while maintaining said pressure.

4. A process of casting aluminum alloyed with from 0.5% to 15% silicon which comprises placing a crucible containing the alloy in molten form, and a mold for receiving said molten alloy, within a pressure chamber, creating a pressure of at least five atmospheres in excess of atmospheric pressure within said chamber, and pouring the molten alloy from the crucible into the mold while maintaining said pressure.

5. A process of casting aluminum alloyed with from 8% to 15% silicon and further treated with sodium which comprises placing a crucible containing the alloy in molten form, and a mold for receiving said molten alloy, within a pressure chamber, creating a pressure of at least five atmospheres in excess of atmospheric pressure within said chamber, and pouring the molten alloy from the crucible into the mold while maintaining said pressure.

6. A process of casting aluminum alloyed with from 0.5% to 15% silicon, manganese, magnesium and alkali metals which comprises placing a crucible containing the alloy in molten form, within a pressure chamber, creating a pressure of at least five atmospheres in excess of atmospheric pressure within said chamber, and pouring the molten alloy from the crucible into the mold while maintaining said pressure.

JOSEF DORNAUF.